

## UNITED STATES PATENT OFFICE

JOSEPH KENT SMITH, OF DETROIT, MICHIGAN, ASSIGNOR, BY MESNE ASSIGNMENTS, TO  
GRANULAR IRON COMPANY, A CORPORATION OF MICHIGAN

## RAIL STEEL

No Drawing.

Application filed November 24, 1925. Serial No. 71,220.

This invention relates to rail steels and its nature, objects and advantages will be best understood from the following:

It is well known that in plain carbon steels, otherwise of equal quality, wrought and not heat treated, as the percentage of carbon and of manganese rises their strength and rigidity increase, while at the same time their static ductility decreases and their resistance to impact decreases much more rapidly still. As static rigidity and Brinnell hardness increase, so does the resistance to wear in such steels increase. The relation of strength to a given percentage of carbon and/or manganese is relative to the method of steel making employed. In other words, for a given percentage of carbon and/or manganese, steel made by the acid gas open hearth process is somewhat stiffer than is steel made by the basic gas open hearth process and steel made on the electric hearth is stiffer than either.

It is also well known by long experience in rail making that taking such a specification as is in common use for a rail weighing 100 pounds per yard, the carbon percentage should not appreciably exceed .70 per cent (and even at this figure the manganese should be kept below .80 per cent) if the 100 pound rail is to pass the required drop test, which is a commercialized form of impact test, and in which a one ton weight is dropped on the rail from a height of 18 feet. Usually for a 100 pound rail, the works analysis specification calls for from .62 to .75 per cent carbon and from .70 to 1.00 per cent manganese, and it is the common practice as the carbon is raised to come down in the manganese in order to pass the drop test.

With the foregoing brief statement of the standard practice in rail making in mind, it is the object of the present invention, stated in general terms, to obtain either

(a) Greatly increased strength and resistance to wear with a given impact-resistance, or

(b) Greatly increased impact-resistance with a given strength and rigidity.

Stated in other words, I either

(a) May employ percentages of carbon and manganese which would today be regarded

as inordinately high, and secure a steel with greatly increased strength and resistance to wear, which steel, however, will still have approximately the same impact resistance as standard rail steels, or

(b) May employ approximately the same percentages of carbon and manganese as in standard practice, and secure a steel with greatly increased impact resistance, which steel, however, will have approximately the same strength and rigidity as standard rail steels.

I have found that if, in making the steel of my invention, I employ "granular iron" as a base in whole or in part, i.e., iron which has been reduced from its ore without passing thru the molten state, I can obtain the foregoing properties. This iron contains no ferrite-dissolved-nitrides, and if I wish to secure greatly increased strength and resistance to wear, with approximately the same ductility and resistance-impact as in standard rail steels, I increase the carbon-manganese content, and if I desire approximately the same strength and ductility as is customary, with the greater resistance to impact than is the case in standard practice, I employ the usual percentages of the carbon-manganese complex.

As illustrative of the properties of such a rail steel, I have tested rails of the steel as made in the electric furnace and containing .79 per cent carbon and 1.08 per cent manganese. The rails tested to an increase of about 20 per cent in strength, a greatly increased rigidity, and a correspondingly increased hardness, notwithstanding which the rail not only withstood the prescribed drop test with ease but was able to withstand repetitions of the test well beyond the point at which the "softer" or "conventional" rail steel failed. The result obtained with these test pieces was all the more remarkable because the steel was cast into a small ingot and rolled down only to the size of 100 pounds per yard, in consequence of which the bars were not "worked" nearly as extensively as would be the case in normal rail manufacture.

I give as the preferred range of carbon and manganese for rail steel of the foregoing

55

60

65

70

75

80

85

90

95

100

characteristics, carbon from .60 per cent to .90 per cent and manganese from .7 per cent to 1.25 per cent.

The granular iron referred to may be made by the method disclosed in Hornsey application Serial No. 532,486, filed January 28, 1922. The Hornsey method as disclosed in said application discloses a process of reducing iron oxide bearing materials to iron without melting, involving the introduction of the ore in a fine state of division into the upper end of the gas sealed apparatus. The apparatus disclosed includes three rotary cylinders. In the first the ore is preheated to approximately the temperature of reaction. To the preheated ore is added a mixture of solid carbonaceous reducing agent in a fine state of division. The mixture of ore and fine carbonaceous material is passed through a second cylinder in which reduction takes place. The gases from the second or reducing cylinder are passed to the preheating cylinder where they are burned to effect the preheating. The reduced material from the second cylinder is passed to a third cylinder which is preferably water cooled. This cylinder reduces the temperature of the reduced product to such a point that it will not readily reoxidize by exposure to air.

From what has been said it is believed that those skilled in the art will appreciate the advantages of the invention. The invention may be applied to types of steel other than "rail" steel.

What I claim is:

1. Rail steel embodying solid produced iron which is free from ferrite dissolved nitrides as a base and carbon appreciably above .70 percent with manganese not lower than customary for .70 per cent carbon.
2. Rail steel embodying solid produced iron which is free from ferrite dissolved nitrides as a base and carbon appreciably above .70 per cent and manganese appreciably above .80 per cent.

In testimony whereof, I have hereunto signed my name.

J. KENT SMITH.